# EUROPEAN PATENT APPLICATION

(11) **EP 4 775 703 A1**
(43) Date of publication of application: **15.07.2026**
(21) Application number: 24862673.1
(22) Date of filing: 28.08.2024
(51) Int. Cl.: C22C 29/08, B21B 27/00, B22F 5/00, C22C 1/051, C22C 27/04

(54) **CEMENTED CARBIDE**

(30) Priority: 07.09.2023 JP 2023145161
(71) Applicant: Mitsubishi Materials Hardmetal Corporation, Gifu 503-2301 (JP)
(72) Inventor: SHIBUTANI, Naoki, Anpachi-gun, Gifu 503-2301 (JP)
(74) Representative: Gille Hrabal Partnerschaftsgesellschaft mbB Patentanwälte
(86) International application number: PCT/JP2024/030729
(87) International publication number: WO 2025/053021

(57) **Abstract**

A cemented carbide comprises:
8.0 to 28.0 mass% in total Co and Ni, the ratio (mass % of Co)/ (mass % of Ni) being 1.0 to 4.0,
0.5 to 2.5 mass% Cr, 4.2 to 5.7 mass% C, more than 0.0 mass% and not more than 1.0 mass% Zr, and
the balance being W and inevitable impurities, wherein
{(mass% of Zr)/ [(mass% of W) + (mass% of Zr)]} × 100 is in a range of 0.4% to 1.5%,
a composite carbide of Zr and W is contained in the secondary hard phases,
in the primary hard phases, the Zr content is in a range of 0.5 to 1.0 mass% relative to all components of the primary hard phases, and
in the secondary hard phases, the W content is in a range of 25.0 mass% or less relative to all components of the secondary hard phases.

## Description

### Technical Field

The present invention relates to cemented carbide used in tools that induce plastic deformation in workpieces under high temperatures. This application claims priority based on Japanese Patent Application No. 2023-145161, filed on September 7, 2023. The entire contents of the Japanese patent application are incorporated herein by reference.

### Background Art

In cemented carbides used in tools that induce plastic deformation in workpieces under high temperatures, use of WC having a specific range of average grain sizes and/or addition of ZrC or a composite compound of Zr and Hf have been proposed to improve the performance of the tools.

For example, PTL 1 discloses a cemented carbide containing Co alone or combination of Co and Cr₃C₂ in the binder phases, having an average size of WC grains in a range of 0.5 to 6 µm, and containing 2.0 to 20 mass% ZrC or (Zr,Hf)C relative to the total amount of the binder phases. This cemented carbide exhibits excellent strength and oxidation resistance at high temperatures.

### Citation List

### Patent Literature

PTL 1: Japanese Unexamined Patent Publication No. 2003-113437

### Summary of Invention

### Technical Problem

An object of the present invention, which has been accomplished in light of the aforementioned circumstances and proposals, is to produce a highly durable cemented carbide for use in tools that induce plastic deformation to workpieces at high temperatures (e.g., hot working temperatures of steel).

### Solution to Problem

A cemented carbide according to an embodiment of the present invention comprises:
8.0 to 28.0 mass% in total Co and Ni, the ratio (mass % of Co)/ (mass % of Ni) being 1.0 to 4.0,
0.5 to 2.5 mass% Cr, 4.2 to 5.7 mass% C, more than 0.0 mass% and not more than 1.0 mass% Zr, and
the balance being W and inevitable impurities, wherein
{(mass% of Zr)/ [(mass% of W) + (mass% of Zr)]} × 100 is in a range of 0.4 to 1.5,
the cemented carbide comprises binder phases, primary hard phases, and secondary hard phases, wherein
   Co and Ni are the main components of the binder phases,
   W is the main component of the primary hard phases in the form of carbide,
   a composite carbide of Zr and W is contained in the secondary hard phases,
   in the primary hard phases, the Zr content is in a range of 0.5 to 1.0 mass% relative to all components of the primary hard phases, and
   in the secondary hard phases, the W content is in a range of 25.0 mass% or less relative to all components of the secondary hard phases.

The cemented carbide may satisfy one or more of the following conditions (1) and (2):
(1) In the primary hard phase, (number of Zr atoms) / [(number of Zr atoms) + (number of W atoms)] × 100 is 1.5 to 2.5.
(2) At the grain boundaries between the main components constituting the binder phases, the fraction of grain boundaries where elements other than Co and Ni segregate is 30% or less.

### Advantageous Effects of Invention

The cemented carbide of the embodiments is a material exhibiting improved durability suitable for a tool inducing plastic deformation to workpieces under high temperatures.

### Brief Description of Drawing

Figure 1 is a schematic cross-sectional view of an apparatus for thermal load testing simulating hot rolling.
Figure 2 is a schematic diagram illustrating the heating zone (heating width) of a hollow cylindrical sintered compact simulating a hot mill roll in the apparatus of Figure 1.

### Description of Embodiments

The inventor has diligently investigated measures of enhancing the durability of cemented carbide used in tools that induce plastic deformation to workpieces under high temperatures, particularly cemented carbide used in hot mill rolls.

As a result, the inventor has recognized that mere measures to problems, such as a reduction in strength at high temperatures and oxidation resistance of cemented carbide, have limitations in improving durability. To overcome these limitations, properties that inhibit the propagation of cracks caused by thermal fatigue, particularly the mesh cracks (cracks propagating in multiple directions on the surface of hot-rolled rolls) that form on the surface during use of hot-rolled rolls.

Upon further investigation, the inventor has discovered that addition of a specified amount of Zr to cemented carbide can inhibit the propagation of mesh cracks.

The cemented carbide according to the embodiments of the present invention will now be described.

Throughout the description of the specification and the claims, a numerical range expressed as "L to M" (where L and M are both numerical values), is synonymous with "L or more and M or less." This range includes both the upper limit (M) and the lower limit (L). If only the upper limit (M) is given a unit, the upper limit (M) and the lower limit (L) has the same unit. The secondary hard phase in this embodiment may also be referred to as the γ phase.

### 1. Composition

The composition will now be described.

### (1) Co and Ni

It is preferred that the total content of Co and Ni be 8.0 to 28.0 mass%. At a total content of Co and Ni less than 8.0 mass%, the cemented carbide exhibits low toughness; whereas at a content exceeding 28.0 mass%, the cemented carbide fails to exhibit the specified hardness.

The addition of Ni, as well as Co increases oxidation resistance at high temperatures, facilitates the binder phases maintaining their fcc crystal structure, suppresses transformation from the fcc crystal structure to other crystal structures, and prevents strain associated with such transformation. To suppress this strain, it is preferred that the ratio (Co mass%) / (Ni mass%) be 1.0 to 4.0, more preferably 2.0 to 3.0.

### (2) Cr

It is preferable for Cr to be present at 0.5 to 2.5 mass %.

Cr dissolves in the binder phases, suppresses the growth of W carbides contained in the primary hard phases, and refines grains of the W carbides. As a result, the composition exhibits desirable oxidation resistance, toughness, and strength to the cemented carbide.

At a Cr content less than 0.5 mass%, the cemented carbide exhibits low oxidation resistance. At a content exceeding 2.5 mass%, Cr surpasses the solubility limit in the binder phases, causing aggregation and thus a reduction in the toughness of the cemented carbide. A preferred Cr content is in a range of 0.8 to 2.0 mass%.

### (3) C

C is compounded to form carbides and is exclusively contained in the primary hard phases and secondary hard phases. The content is preferably in a range of.4.2 mass% to 5.7 mass%. Within this range, sufficient amounts of carbides are formed in the primary hard phases and secondary hard phases.

### (4) Zr

Zr is compounded to ensure of uniform dispersion of the binder phases and to suppress the propagation of mesh cracks. The Zr content is preferably in the range of greater than 0.0 mass% and less than 1.0 mass%. More preferably, the Zr content is in the range of 0.1 mass% to 0.9 mass%.

Regarding the entire alloy, it is preferred that the ratio {(Zr mass%) / [(W mass%) + (Zr mass%)]} × 100 is within a range of 0.4 to 1.5.

A mass fraction within such a range leads to suppression of the propagation of mesh cracks under high temperatures. The reason for selecting this mass ratio is that a fraction below 0.4% result in non-uniform dispersion of binder phases, while a fraction exceeding 1.5% cause increased crack formation due to agglomeration of secondary hard phases.

This mass fraction is in a range of more preferably 0.5% to 1.3%, even more preferably 0.7% to 1.2%.

### (5) W

W is the main component of the primary hard phases. All constituents of the primary hard phases contain at least 50 atomic percent W carbides (primarily WC, but may also include other W carbides not limited to stoichiometric composition). The W content also has a preferred value within the secondary hard phases, as described later.

### (6) Ti, V, Nb, Ta, and Mo

It is preferred that the elements Ti, V, Nb, Ta, and Mo are not present; however, their presence is permissible as inevitable impurities as described later.

### (7) Segregation of elements at boundaries between crystal grains of the main components constituting the binder phases

It is more preferred that the fraction of grain boundaries where uneven concentration peaks of elements (such as Cr or W) other than Co and Ni are observed (i.e., segregation occurs) at the boundaries between crystal grains of the main components, namely, Co, Ni, and the Co-Ni solid solution, constituting the binder phases is 30% or less for the following reasons. A fraction exceeding 30% causes precipitates at the grain boundaries to reduce the strength of the grain boundaries, making them prone to become crack propagation paths. An ideal lower limit for this fraction of grain boundaries is 0%. Following an exemplary process described later results in a lower limit of approximately 10%.

### (8) Inevitable Impurities

Inevitable impurities that are unintentionally introduced during the manufacturing process may be present in the primary hard phases, secondary hard phases, and binder phases. Examples of the inevitable impurities include Fe, N, O, and Hf. The total amount of inevitable impurities, expressed as an external amount relative to the entire cemented carbide being 100 mass%, should preferably be 0.3 mass% or less.

### 2. Microstructure

The microstructure of the alloy will now be described.

### (1) Binder phase

The binder phases each have an fcc or hcp crystal structure.

The main components of binder phases are Co and Ni. In other words, Co and Ni together occupy at least 50 atomic percent of the elements contained in the binder phases.

In addition to Co and Ni, binder phases may contain Cr, W and C, which are the main constituents of the hard phases, and inevitable impurities. These components, if present in binder phases, are presumed to be in a state of solid solution within the binder phases. Note that Zr is essentially absent in binder phases (present in amounts below the detection limit).

### (2) Secondary hard phase

The secondary hard phases each have an fcc crystal structure.

The main component of the secondary hard phases is Zr carbides (not limited to stoichiometric composition). The term "main component" indicates that Zr carbides occupy 50 atomic % or more of all elements contained in the secondary hard phases. In addition to Zr carbides, the secondary hard phase may also contain Cr, W and C from the primary hard phases, Co and Ni from the binder phases, and inevitable impurities.

The W content is preferably less than 25.0 mass% of all components contained in the secondary hard phases, to suppress the reaction between Zr and W and to inhibit the propagation of mesh cracks (although the lower limit is approximately 2.0 mass% in one exemplary process described later, it may be 0.0 mass%).

The number of W atoms contained in the secondary hard phase is preferably within the range of 6.0 mass% to 12.0 mass% of the sum of the numbers of Zr and W atoms contained in the secondary hard phases, namely: <W>/(<W> + <Zr>) × 100 (where <W> and <Zr> represent the numbers of W and Zr atoms, respectively). Satisfying this range further reliably suppresses the propagation of mesh cracks.

Although the secondary hard phases may have any average primary grain size without any particular constraints, a grain size of 0.5 µm or greater and less than 1.5 µm is more preferable. An average grain size less than 0.5 µm causes the surface area of the secondary hard phases to increase, potentially causing precipitation of ZrO₂ during sintering. An average grain size of 1.5 µm or greater causes excessively large secondary hard phases to be formed, making it easier for binder pools, which are aggregates of binder phases, to form. This behavior increases the distance between primary hard phases, potentially reducing strength. The average primary grain size of the secondary hard phases is preferably in the range of 0.6 to 1.3 µm. The definition of the average primary grain size of the secondary hard phases is described later.

### (3) Primary hard phase

The primary hard phases each have a hexagonal close-packed (hcp) crystal structure.

The primary hard phases contain the main component of tungsten carbide (tungsten carbide occupies at least 50 atomic % of all the elements forming the primary hard phases). The primary hard phases may contain components of the binder phases, chromium, and inevitable impurities introduced unintentionally during the manufacturing process. The Zr content in the primary hard phases is preferably 0.5 to 1.0 mass% of all the components contained in the primary hard phases, because Zr removes oxides present at the interface between the primary hard phases and the binder phases, thereby improving durability of a tool made of this cemented carbide and used under high-temperature conditions. The Zr content in the primary hard phases is more preferably 0.6 to 0.9 mass%.

The Zr content (number of Zr atoms) within the primary hard phases is preferably 1.5% to 2.5% of the total number of Zr and W atoms within the primary hard phases, i.e., <Zr>/(<Zr>+<W>) × 100 (where <Zr> and <W> represent the numbers of Zr and W atoms, respectively). Satisfying this range further reliably suppresses the propagation of mesh cracks.

Although the primary hard phases have any average grain size without particular constraints, a size in the range of 2.0 to 9.0 µm is preferred. A size below 2.0 µm may cause the toughness of the cemented carbide to decrease, while a size exceeding 9.0 µm may cause the hardness to decrease. The average grain size of the primary grains in the primary hard phases is more preferably 3.0 µm to 8.0 µm, even more preferably 4.0 µm to 6.0 µm. The definition of the average size of the primary grains in the primary hard phases is described later.

### (4) Ratio of average primary grain size of primary hard phases to secondary hard phases

The ratio of average primary grain size of the primary hard phases to the secondary hard phases, namely (average primary grain size of primary hard phases) / (average primary grain size of secondary hard phases), is preferably in the range of 4.0 to 5.0. A ratio falling within this range leads to generation of finer mesh cracks during hot working in both primary hard phases and secondary hard phases. This behavior avoids concentration of thermal stress at specific cracks and more effectively suppresses the formation of deep cracks.

### 3. Measurement of average particle size of primary grains

The grain size of primary grains in the secondary hard phases and primary hard phases is measured as the equivalent circular diameter, i.e., the diameter (D50) of a circle with an area equal to the area of the secondary hard phase or primary hard phase, as follows:
(1) An arbitrary surface or cross-section of the cemented carbide is processed to remove fine irregularities to yield a smooth surface that does not interfere with measurement by a backscattered electron diffraction (EBSD) system. Several fields of view, each with dimensions of, for example, 190 µm (vertical) by 242 µm (horizontal) in size are selected on the processed surface. Each field of view is observed with a scanning electron microscope (SEM) equipped with an energy-dispersive X-ray spectrometer (EDS) and EBSD at an acceleration voltage of 15 kV, with an observation point spacing of 0.1 µm, to simultaneously acquire the EBSD pattern and EDS data.

The number of phases to be observed may be the same or different for distinguishing the binder phases, secondary hard phases, and primary hard phases. Preferably, the number is 300 or more, preferably 300 to 1000 for each phase, and the observation field of view is increased until 300 or more phases are observed.

Furthermore, the surface or cross-section may be processed, for example, a focused ion beam (FIB) system.

(2) The results of EBSD measurements and EDS count values are averaged to determine the composition of each phase.

(3) Each phase is identified in accordance with the definitions based on the crystal structure and composition described above. Specifically, the phases having an hcp structure and containing the main component of W carbide from the EBSD pattern are identified as primary hard phases. EDS count values for Co and Ni detected from all the observation points identified as either an fcc or hcp phase are then averaged. Observation points identified as the fcc phase with EDS counts for Co and Ni higher than the average value are identified as the binder phases, while the remainder of the fcc phases is identified as the secondary hard phases.

(4) If adjacent observation points belong to the same phase and have a difference in orientation of 5 degrees or more, the midpoint between these two observation points is determined to be the phase boundary.

(5) The average grain size of each phase is determined by calculation of the areas of 300 or more grains, preferably 300 to 1000 grains, and then calculation of the diameter of a circle with an equal area.

(6) Each phase identified as the primary hard phase or secondary hard phase in Procedure (3) is subjected to EDS measurement again to confirm that the phase identified as the primary hard phase contains at least 50 atomic % W carbide, and that the phase identified as the binding phase contains at least 50 atomic % Co and Ni in total.

(7) Based on the results of Procedures (5) and (6), two graphs are plotted for the grain size of the primary hard phases and the secondary hard phases, respectively, where horizontal axis represents grain size. The vertical axis represents [(Cumulative number of primary hard phases up to each grain size) / (Total number of primary hard phases)] × 100 and [(Cumulative number of secondary hard phases up to each grain size) / (Total number of secondary hard phases)] × 100). The particle size at which the cumulative number percentage reaches 50% is defined as the average grain size (median grain size) (D50).

### 4. Determination of Content of Each Component in Overall Cemented Carbide

The total content of W, Co, Ni, Zr, Cr, and C in the cemented carbide may be determined based on the composition of each phase (the fraction of each component in each phase) and the area fraction of each phase as described above, or may be measured with an electron probe microanalyzer (EPMA). In EPMA measurements, any surface or cross-section of the cemented carbide is smoothed by removing minute irregularities so as not to interfere with EPMA measurement. The mirror-polished surface is irradiated with electron beams inside the EPMA. Each component in the sample is identified and determined from characteristic X-rays emerging from an observation field with dimensions of 512 µm (vertical) by 512 µm (horizontal). Each content is an averaged value.

### 5. Percentage of interfaces exhibiting segregation of elements other than Co at interfaces between binder phases

The percentage of interfaces where elements (such as Cr or W) other than Co segregate at interfaces between binder phases is measured as follows.

For example, several (preferably five or more) fields of view with dimensions of 190 µm (vertical) by 242 µm (horizontal) are selected. Within each field of view, boundaries of binder phases i.e., interfaces between the binder phases and the primary or secondary hard phases are inferred based on images of a dark-field scanning electron microscope (BF-STEM) and of a high-angle annular dark-field scanning transmission electron microscope (HAADF-STEM). EDS line analysis is then performed based on these inferred results. This EDS line analysis definitively determines whether segregation exists at the interface by the presence of concentration peaks for elements other than Co.

The percentage of interfaces showing segregation of elements other than Co at the interface between the binder phases is calculated as: (number of interfaces with segregation) / (total number of interfaces measured) × 100.

The field of view may be either the field of view used to identify the binder phases or a separately selected field of view.

### 6. Production

The cemented carbide according to this embodiment can be manufactured, for example, as follows:

The raw material powders of WC, Co, Ni, Cr₃C₂, and ZrC are compounded in predetermined proportions. The mixture is then pulverized and mixed in an attritor, followed by vacuum drying to yield blended raw material.

The blended raw material is then pressed into a green compact with a specified shape. Under vacuum conditions, the green compact undergoes multiple cycles of heating and temperature holding to ensure uniform heating throughout all parts of the green compact to a sintering temperature of 1300°C to 1400°C, and then held at the sintering temperature for 30 to 90 minutes.

After sintering is complete, the sintered compact is slowly cooled over 1.5 to 5 hours until the compact reaches a predetermined temperature between 900 and 1100°C, where the predetermined temperature and cooling time depend on the shape of the compact (The reason for the varying cooling times is that this cooling is performed while applying electrical heating, resulting in an inconsistent cooling rate). Once the compact reaches the target cooling temperature, it is subjected to rapid cooling to room temperature by injection of argon gas.

The temperature is then raised again to 1250 to 1350°C, and the compact is subjected to HIP treatment under an Ar gas atmosphere, and then is slowly cooled over 5.5 to 8.5 hours from 600 to 400°C while undergoing electrical heating.

The above explanation includes the following features:

### (Appendix 1)

A cemented carbide comprising:
8.0 to 28.0 mass% in total Co and Ni, the ratio (mass of Co)/ (mass of Ni) being 1.0 to 4.0,
0.5 to 2.5 mass% Cr, 4.2 to 5.7 mass% C, more than 0.0 mass% and not more than 1.0 mass% Zr, and
the balance being W and inevitable impurities, wherein
{(mass% of Zr)/ [(mass% of W) + (mass% of Zr)]} × 100 is in a range of 0.4 to 1.5,
the cemented carbide comprises binder phases, primary hard phases, and secondary hard phases, wherein
   Co and Ni are the main components of the binder phases,
   W is the main component of the primary hard phases in the form of carbide,
   a composite carbide of Zr and W is contained in the secondary hard phases,
   in the primary hard phases, the Zr content is in a range of 0.5 to 1.0 mass% relative to all components of the primary hard phases, and
   in the secondary hard phases, the W content is in a range of 25.0 mass% or less relative to all components of the secondary hard phases.

### (Appendix 2)

The cemented carbide described in Appendix 1, wherein in the primary hard phases, the fraction (number of Zr atoms) / [(number of Zr atoms) + (number of W atoms)] × 100 is 1.5 to 2.5.

### (Appendix 3)

The cemented carbide as described in Appendix 1 or 2, wherein the fraction of grain boundaries where elements other than Co and Ni segregate in the grain boundaries between crystal grains of the main components constituting the binder phases is 30% or less.

### (Appendix 4)

The cemented carbide as described in any one of Appendices 1 to 3, wherein the ratio (the average size of the primary grains of the primary hard phases) / (the average size of the primary grains of the secondary hard phases) is 4.0 to 5.0.

### (Appendix 5)

The cemented carbide as described in any one of Appendices 1 to 4, wherein in the secondary hard phases, the fraction (number of W at oms) / [(number of W atoms) + (number of Zr atoms)] × 100 is 6.0 to 12.0

### (Appendix 6)

The cemented carbide as described in any one of Appendices 1 to 5 wherein the average grain size of the secondary hard phases is 0.5 µm or more and less than 1.5 µm.

### (Appendix 7)

The cemented carbide as described in any one of Appendices 1 to 6, wherein the average grain size of the primary hard phases is 2.0 to 9.0 µm.

### Examples

The cemented carbide of the present invention will now be described in detail by way of examples of hollow cylindrical sintered compact fabricated to simulate a hot mill roll in detail. However, the present invention is construed not limiting the examples.

### 1. Production on Examples and Comparative Examples

Sintered compacts simulating hot mill rolls with the cemented carbide compositions shown in Table 3 (Examples 1 to 14 and Comparative Examples 1' to 9') were prepared as follows:

### (1) Raw Material Powders and Mixing Step

The following raw material powders were prepared for sintered compacts of cemented carbide: WC powder (FSSS diameter: 6.2 µm), Co powder (FSSS diameter: 1.5 µm), Ni powder (average particle size D50: 0.8 µm), Cr₃C₂ powder (FSSS diameter: 3.3 µm), and ZrC powder (FSSS diameter: 2.4 µm).

The average particle size D50 of the Ni powder is the median diameter determined as a volume fraction from measurements with a laser particle size distribution analyzer.

These powders were blended in the formulations shown in Table 1 and pulverized and mixed in an attritor.

### (2) Sintering Step

The mixed powder was dried and pressed at 100 MPa to form a hollow cylindrical shape with an outer diameter of 50 mm, an inner diameter of 18 mm, and a height of 37 mm, yielding the molded compact. Subsequently, under a vacuum of 1 Pa or less, the heating and temperature holding cycles were repeated until it could be considered that all parts of the molded compact had heated uniformly (at the same rate) up to 1250°C. Sintering was then performed under the conditions shown in Table 2. After sintering, the compact was electrically cooled at a rate of 1.5 to 1.6°C/min for 5 hours to a target cooling temperature of 900°C, then rapidly cooled to room temperature with Ar gas. Subsequently, the compact was reheated to 1290°C, subjected to HIP treatment at 88.3 MPa under an Ar gas atmosphere, and then electrically heated over 7 hours while being slowly cooled to 500°C. The sintered compact was then machined into a hollow cylindrical shape with an outer diameter of 40 mm, an inner diameter of 16 mm, and a height of 30 mm.

The reason for the range in the electrical cooling rate is that maintaining a constant electrical cooling rate was difficult.

**[Table 1]**

| Type | | Composition (mass%) | | | | | |
|---|---|---|---|---|---|---|---|
| | | Co | Ni | Co+Ni | Cr₃C₂ | ZrC | WC |
| Example | 1 | 22.0 | 5.5 | 27.5 | 2.0 | 0.9 | Balance |
| | 2 | 11.0 | 5.5 | 16.5 | 1.5 | 0.5 | Balance |
| | 3 | 11.0 | 5.5 | 16.5 | 1.5 | 0.4 | Balance |
| | 4 | 11.0 | 5.5 | 16.5 | 1.5 | 0.7 | Balance |
| | 5 | 11.0 | 5.5 | 16.5 | 1.5 | 0.9 | Balance |
| | 6 | 17.0 | 8.5 | 25.5 | 2.2 | 0.3 | Balance |
| | 7 | 17.0 | 8.5 | 25.5 | 2.2 | 0.6 | Balance |
| | 8 | 17.0 | 8.5 | 25.5 | 2.2 | 0.8 | Balance |
| | 9 | 17.0 | 8.5 | 25.5 | 2.2 | 1.1 | Balance |
| | 10 | 18.0 | 4.5 | 22.5 | 1.7 | 0.7 | Balance |
| | 11 | 6.6 | 3.3 | 9.9 | 0.9 | 0.3 | Balance |
| | 12 | 6.6 | 3.3 | 9.9 | 0.9 | 0.8 | Balance |
| | 13 | 12.6 | 6.3 | 18.9 | 1.7 | 0.6 | Balance |
| | 14 | 18.6 | 9.3 | 27.9 | 2.4 | 0.9 | Balance |
| Comparative Example | 1' | 22.0 | 5.5 | 27.5 | 2.0 | 0.0 | Balance |
| | 2' | 11.0 | 5.5 | 16.5 | 1.5 | 0.0 | Balance |
| | 3' | 11.0 | 5.5 | 16.5 | 1.5 | 0.2 | Balance |
| | 4' | 17.0 | 8.5 | 25.5 | 2.2 | 0.0 | Balance |
| | 5' | 17.0 | 8.5 | 25.5 | 2.2 | 1.4 | Balance |
| | 6' | 18.0 | 4.5 | 22.5 | 1.7 | 0.0 | Balance |
| | 7' | 6.6 | 3.3 | 9.9 | 0.9 | 0.0 | Balance |
| | 8' | 12.6 | 6.3 | 18.9 | 1.7 | 0.0 | Balance |
| | 9' | 18.6 | 9.3 | 27.9 | 2.4 | 0.0 | Balance |

**[Table 2]**

| Type | | Sintering temp. (°C) | Sintering time (min) |
|---|---|---|---|
| Example | 1 | 1335 | 60 |
| | 2 | 1360 | 60 |
| | 3 | 1360 | 60 |
| | 4 | 1360 | 60 |
| | 5 | 1360 | 60 |
| | 6 | 1335 | 60 |
| | 7 | 1335 | 60 |
| | 8 | 1335 | 60 |
| | 9 | 1335 | 60 |
| | 10 | 1340 | 60 |
| | 11 | 1370 | 60 |
| | 12 | 1370 | 60 |
| | 13 | 1355 | 60 |
| | 14 | 1330 | 60 |
| Comparative Example | 1' | 1340 | 60 |
| | 2' | 1360 | 60 |
| | 3' | 1360 | 60 |
| | 4' | 1345 | 60 |
| | 5' | 1335 | 60 |
| | 6' | 1345 | 60 |
| | 7' | 1370 | 60 |
| | 8' | 1355 | 60 |
| | 9' | 1340 | 60 |

### 2. Evaluation of Examples and Comparative Examples

### (1) Composition, Average Grain Size

The content of each component and the average grain size of the primary hard phases and secondary hard phases were measured by the aforementioned method. The results are shown in Table 3. In all examples and comparative examples, the content of inevitable impurities was 0.3 mass% or less by extra number, and the Zr content in the binder phase was below the detection limit.

Note that in Table 3, symbol "-" indicates below the detection limit. For some comparative examples where no secondary hard phases exist, "Average grain size of secondary hard phase (D50: µm)" is listed as "Unmeasurable," and "(Primary average particle size of main hard phase)/(Primary average particle size of secondary hard phase)" is listed as "Uncalculable."

### (2) Fraction of grain boundaries containing elements other than Co and Ni to the grain boundaries between the main components constituting the binder phases.

For Example 1 and Comparative Example 1', the fraction of grain boundaries containing elements other than Co and Ni was measured to the grain boundaries between Co crystal grains by the aforementioned method (with five observation fields of view). The EDS line analysis with the STEM were performed at an observation magnification of 738,000, a spot diameter of 132 pm, a spot spacing of 132 pm, a line length of 50 nm, and a measuring points of 400. The results are shown in Table 4. The segregation rate in Table 4 refers to the percentage of grain boundaries containing elements other than Co and Ni having concentration peaks (indicating segregation) at the grain boundaries between the crystalline grains of the main components constituting the aforementioned composite phase, where the concentration peak is determined in the case that the atomic percentage of the element at the location of the peak is at least 1.5 times the atomic percentage of that element elsewhere.

Table 4 evidentially demonstrates that Example 1 exhibits a lower fraction of grain boundaries between crystal grains containing elements other than Co and Ni at the interfaces between the main components constituting the binder phases, compared to Comparative Example 1'.

**[Table 4]**

| Type | Rate of segregation (%) |
|---|---|
| Example 1 | 25 |
| Comparative Example 1' | 60 |

### (3) Thermal Load Test

Sintered compacts with an outer diameter of 40 mm, an inner diameter of 16 mm, and a height (roll width when viewed as a mill roll) of 30 mm, shaped as hollow cylinders simulating hot-mill rolls, have compositions corresponding to Example 1 and Comparative Example 1'. These compacts were subjected to a thermal load test simulating hot rolling, involving repeated heating and cooling cycles, followed by evaluation of mesh cracks.

The apparatus for the thermal load test conformed to that described in Int. Journal of Refractory Metals and Hard Materials 60 (2016) pp. 118-124. With reference with Figure 1, this sintered cemented carbide compact (1) with a hollow cylindrical shape was rotated at 4 rpm in the direction of the arrow. A heating-cooling cycle was repeated 3000 times: heating to 600°C with a high-frequency coil over approximately one-quarter of a revolution (2), followed by water cooling in the cooling water spray region (3). The heating width (5) was limited to only the central 10 mm (see Figure 2). The cooling water was sprayed so as not to flow into the high-frequency coil and was recovered in the water tank (4).

The thermal load imparting this heating-cooling cycle simulates the thermal cycle of mill rolls during actual hot rolling.

Specifically, during hot rolling, the portion of the mill rolls in contact with the rolled material absorbs heat from the material and becomes hot, while the two ends not in contact with the rolled material are not heated and are cooled by cooling water.

The reason for setting the heating temperature to 600°C is that a heating temperature exceeding 600°C causes the WC to oxidize, rendering it unusable as a mill roll; hence, the mill rolls are supposed not to exceed 600°C during hot rolling.

After completing this thermal load test, the sintered compact of the cemented carbide in the shape of a hollow cylinder was cut radially to include the heated center (the central part in the height direction of the hollow cylinder). The length of the cracks that developed on the cross-section was then measured in accordance with the following procedure.
1) The two ends of the outer periphery of the heating region (corresponding to the outer circumference at a central angle of 1.8 degrees of the hollow cylindrical compact) were positioned on a diagonal of a rectangular observation field measuring approximately 450 µm long and 630 µm wide, which are magnified 200 times.
2) Starting from one end of the outer peripheral portion and extending toward the other end, peripheral points were set on the outer peripheral portion at 100 µm intervals parallel to the diagonal.
3) These peripheral points were connected by a straight line using least squares approximation, and this line was defined as the perimeter line for measuring crack length.
4) A straight line is drawn parallel to this perimeter line passing through the deepest point of the crack (the point closest to the radial center of the hollow cylinder). The distance between this line and the outer circumference line is measured, and treated as the crack length. Cracks with lengths of 200 µm or greater were observed at a magnification of 100. Cracks with lengths of 10 µm or less were ignored.

The observation magnification is set to 100. However, cracks longer than 200 µm may extend beyond the field of view, precluding measurement of their full length; hence, the magnification of 100 is mere a guideline; the magnification was adjusted depending on the crack length to be measured.

Cracks shorter than 10 µm were excluded from observation. These cracks are thinner than the oxide layer formed on the mill roll surface and are presumed to have been generated by spalling rather than thermal cycling.

Table 4 shows the results of measurement. The average crack length in Table 4 is the mean value of the measured crack lengths.

### (4) Fracture Toughness

The fracture toughness was measured by a Single Edge V-Notch Beam method (SEVNB method).

A cubic sintered compact was fabricated with the same composition and under the same manufacturing conditions as in Examples 1 and 2. From this sintered compact a 3 by 4 by 40 mm strip-shaped test specimen was prepared. A V-notch with a depth of 1.5 mm, a perpendicularity of 0.01 mm or less, and a tip radius of 15 µm was machined at the longitudinal center. A flexural strength test was then conducted. For testing, the specimen was positioned so that the V-notch aligned with the center of the two pins of the three-point bneding setup. Testing was conducted in air at 1000^{∘}C with a span length of 16 mm and a load cell loading rate of 0.5 mm/min.

The results are shown in Table 5.

**[Table 5]**

| Type | Corresponding Comparative Example | Heat Load Test | | Fracture toughness | |
|---|---|---|---|---|---|
| | | Average crack depth (µm) | Ratio of average crack depth to corresponding Comparative Example | 1000°C [MPa m^{1/2}] | Ratio of fracture toughness to corresponding Comparative Example |
| Example 1 | 1 | 87.36 | 0.72 | 23.60 | 1.48 |
| Example 2 | 2 | 36.41 | 0.50 | 18.90 | 1.11 |
| Example 3 | 2 | 40.51 | 0.55 | 17.60 | 1.04 |
| Example 4 | 2 | 33.48 | 0.46 | 19.60 | 1.15 |
| Example 5 | 2 | 37.95 | 0.52 | 19.40 | 1.14 |
| Example 6 | 4 | 49.82 | 0.52 | 17.40 | 1.07 |
| Example 7 | 4 | 48.62 | 0.51 | 18.80 | 1.16 |
| Example 8 | 4 | 73.48 | 0.77 | 20.20 | 1.25 |
| Example 9 | 4 | 75.96 | 0.79 | 19.10 | 1.18 |
| Example 10 | 6 | 65.35 | 0.74 | 18.20 | 1.04 |
| Example 11 | 7 | 14.24 | 0.83 | 17.40 | 1.04 |
| Example 12 | 7 | 13.24 | 0.77 | 18.60 | 1.11 |
| Example 13 | 8 | 31.04 | 0.49 | 16.90 | 0.87 |
| Example 14 | 9 | 41.72 | 0.50 | 16.00 | 0.68 |
| Comparative Example 1' | - | 120.56 | - | 16.00 | - |
| Comparative Example 2' | - | 73.41 | - | 17.00 | - |
| Comparative Example 3' | 2' | 64.52 | 0.88 | Not measured | - |
| Comparative Example 4' | - | 95.86 | - | 16.20 | - |
| Comparative Example 5' | 4' | 358.90 | 3.74 | Not measured | - |
| Comparative Example 6' | - | 88.09 | - | 17.50 | - |
| Comparative Example 7' | - | 17.22 | - | 16.80 | - |
| Comparative Example 8' | - | 62.81 | - | 19.50 | - |
| Comparative Example 9' | - | 83.51 | - | 23.40 | - |

In Table 5, "Corresponding Comparative Example" indicates the number of the Comparative Example that has the same contents of alloy components other than Zr but does not contain Zr.

Columns for "Ratio of average crack depth to corresponding Comparative Example" and "Ratio of fracture toughness to corresponding Comparative Example" demonstrate that Examples exhibit a smaller average crack depth and higher fracture toughness due to an appropriate Zr content. In the column for "Ratio of average crack depth to corresponding Comparative Example," Comparative Examples 3' and 5' contain 0.2 wt% and 1.2 wt% Zr, respectively, and show the ratio of average crack depth to corresponding Comparative Examples 2' and 4'. The "Ratio of average crack depth to corresponding Comparative Example" for Comparative Examples 3' and 5' demonstrates that an improper Zr content leads to a deeper average crack depth.

### (4) Regrinding depth Test

Rolls with an outer diameter of 283.5 mm, an inner diameter of 160 mm, and a length of 70 mm were manufactured with the composition of Example 2 and Comparative Example 2' under the same manufacturing conditions as Example 2 and Comparative Example 2'. These rolls were subjected to rolling under the following hot working conditions.
Caliber shape: Elliptical (width 33.33 mm, depth 5.5 mm, caliber R 28 mm, shoulder an r 3 mm caliber)
Rolled Material: A combination of SCM435 and SUM24L to achieve the total rolled material mass
Rolling Temperature: 500°C
Total Rolled Material Mass: 4400 tons
The regrinding depth is shown in Table 6.

The regrinding depth refers to the amount of material removed by regrinding a roll to restore it for reuse after surface roughness and internal cracks developed from use. A high average regrinding depth accordingly indicates that the surface roughness and internal cracks caused by roll usage are more severe.

**[Table 6]**

| Type | Regrinding depth (mm) |
|---|---|
| Example 2 | 1.08 |
| Comparative Example 2' | 1.41 |

Table 6 shows that the regrinding depth for Example 2 is less than that for Comparative Example 2', can be reground more times before reaching the scrap diameter, and thus has a longer service life in use as a roll.

The embodiments disclosed above are merely illustrative in all respects and are not intended to be limiting. The scope of the present invention is defined by the appended claims, not by the embodiments described above, and it is intended to include all modifications within the gist and scope of the claims and equivalents.

### Reference Signs List

1 Hollow cylindrical sintered compact simulating hot mill roll
2 Heating zone using high-frequency coils
3 Cooling water spray zone
4 Water tank
5 Heating width

## Claims

1. A cemented carbide comprising:
8.0 to 28.0 mass% in total Co and Ni, the ratio (mass% of Co)/ (mass% of Ni) being 1.0 to 4.0,
0.5 to 2.5 mass% Cr, 4.2 to 5.7 mass% C, more than 0.0 mass% and not more than 1.0 mass% Zr, and
the balance being W and inevitable impurities, wherein
{(mass% of Zr)/ [(mass% of W) + (mass% of Zr)]} × 100 is in a range of 0.4 to 1.5,
the cemented carbide comprises binder phases, primary hard phases, and secondary hard phases, wherein
Co and Ni are the main components of the binder phases,
W is the main component of the primary hard phases in the form of carbide,
a composite carbide of Zr and W is contained in the secondary hard phases,
in the primary hard phases, the Zr content is in a range of 0.5 to 1.0 mass% relative to all components of the primary hard phases, and
in the secondary hard phases, the W content is in a range of 25.0 mass% or less relative to all components of the secondary hard phases.

2. The cemented carbide described in Claim 1, wherein in the primary hard phases, the fraction (number of Zr atoms) / [(number of Zr atoms) + (number of W atoms)] × 100 is 1.5 to 2.5.

3. The cemented carbide as described in Claim 1 or 2, wherein the fraction of grain boundaries where elements other than Co and Ni segregate in the grain boundaries between crystal grains of the main components constituting the binder phases is in a range of 10% to 30%.
